# EUROPEAN PATENT SPECIFICATION

(11) **EP 1 759 056 B1**
(45) Date of publication and mention of the grant of the patent: **27.08.2008**
(21) Application number: 05744423.4
(22) Date of filing: 31.05.2005
(51) Int. Cl.: D21G 1/00, D21H 25/06

(54) **METHOD FOR TREATING A FIBROUS WEB DOWNSTREAM OF SLITTING**
VERFAHREN ZUR BEHANDLUNG EINER FASERSTOFFBAHN NACH DEM ZERTEILEN
PROCEDE DE TRAITEMENT DE BANDE FIBREUSE EN AVAL DE L'OPERATION DE REFENTE

(30) Priority: 24.06.2004 FI 20045243
(43) Date of publication of application: 07.03.2007
(73) Proprietor: Metso Paper, Inc.(Reg.No. 763281), 00130 Helsinki (FI)
(72) Inventor: PIETIKÄINEN, Reijo, FI-04420 Järvenpää (FI); SUOMI, Eero, FI-13210 Hämeenlinna (FI); TASKINEN, Pekka, FI-40520 Jyväskylä (FI); VILJANMAA, Mika, FI-00760 Helsinki (FI); VAITTINEN, Henri, FI-04400 Järvenpää (FI); TALJA, Risto, FI-40800 Vaajakoski (FI); NISSINEN, Vilho, FI-04660 Numminen (FI); LAAPOTTI, Jorma, FI-40270 Palokka (FI); ILOMÄKI, Jari, FI-40270 Palokka (FI); LEPOLA, Maria, FI-02170 Espoo (FI); LIPPONEN, Juha, FI-04400 Järvenpää (FI)
(74) Representative: TBK-Patent
(86) International application number: PCT/FI2005/050184
(87) International publication number: WO 2006/000633

(56) References cited:
- WO-A1-03/064761
- WO-A1-03/064764
- FI-B- 81 158

## Description

The present invention relates to a method for treating a fibrous web downstream of slitting, said treatment comprising e.g. calendering, coating or various combinations thereof.

FI-B-81158 discloses a method for treating a fibrous web downstream of slitting and prior to pointing. A wide variety of paper and board grades exist and can be divided according to basis weight in two classes: papers of a single ply with a basis weight of 25-300 g/m² and boards produced by multilayer technique with a basis weight of 150-600 g/ m². As noted, the borderline between paper and board is floating, the boards with lowest basis weight being lighter than the heaviest papers.

The following representative descriptions are examples of currently employed values for fibrous webs and substantial deviations from such values are possible. The main source for descriptions is the publication Papermaking Science and Technology, section Papermaking Part 3, finishing, edit. Jokio M., publ. Fapet Oy, Jyväskylä 1999, page 361.

Mechanical pulp based or wood containing printing papers include newsprint, uncoated magazine and coated magazine paper.

Newsprint consists either entirely of mechanical pulp or may contain a small amount of bleached softwood pulp (0-15%), and/or recycled pulp can be used for replacing some of the mechanical pulp. The following values can probably be considered common for newsprint: basis weight 40-48.8 g/ m², ash content (SCAN-P 5:63) 0-20%, PPS s10 roughness (SCAN-P 76-95) 3.0-4.5 µm, Bendtsen roughness (SCAN-P21:67) 100-200 ml/min, density 600-750 kg/ m³, brightness (ISO 2470:1999) 57-63%, and opacity (ISO 2470:1998) 90-96%.

Uncoated magazine paper (SC = supercalendered) generally comprises mechanical pulp at 50-70%, bleached softwood pulp at 10-25%, and fillers at 15-30%. Typical values for calendered SC paper (including, among others, SC-C, SC-B and SC-A/A+) are basis weight of 40-60 g/ m², ash content (SCAN-P5:63) of 0-35%, Hunter gloss (ISO/DIS 8254/1) of <20-50%, PPS s1 0 roughness (SCAN-P 76:95) of 1.0-2.5 µm, density of 700-1250 kg/m³, brightness (ISO 2470:1999) of 62-70%, and opacity (ISO 2470:1998) of 90-95%.

Table 1 presents typical values for mechanical pulp containing, coatable papers. (MFC = machine finished coated, FOO = film coated offset, LWC = light weight coated, MWC = medium weight coated, HWC = heavy weight coated).

**Table 1**

| | MFC | FOO | LWC | MWC | HWC |
|---|---|---|---|---|---|
| basis weight (g/ m²) | 50-70 | 40-70 | 40-70 | 70-90 | 100-135 |
| Hunter gloss (ISO/DIS 8254/1), (%) | 25-40 | 45-55 | 50-65 | 65-70 | |
| PPS-s10 roughness, (µm) (SCAN-P 76/95) | 2.2-2.8 | 1.5-2.0 | 0.8-1.5 (offset) 0.6-1.0 (roto) | 0.6-1.0 | |
| density, (kg/ m³) | 900-950 | 1000-1050 | 1100-1250 | 1150-1250 | |
| brightness (ISO 2470:1999), (%) | 70-75 | 70-75 | 70-75 | 70-75 | |
| opacity (ISO 2470:1998), (%) | 91-95 | 91-95 | 89-94 | 89-94 | |

Coated magazine paper (LWC = light weight coated) contains mechanical pulp at 40-60%, bleached softwood pulp at 25-40%, and fillers and coating agents at 20-35%.

HWC can be coated even more than twice.

Woodfree printing papers made of chemical pulp or fine grade papers include uncoated - and coated - chemical pulp based printing papers, in which the fraction of mechanical pulp is less than 10%.

Uncoated printing papers based on chemical pulp (WFU) contain bleached birchwood pulp at 55-80%, bleached softwood pulp at 0-30%, and fillers at 10-30%. WFU shows wide fluctuation of values: basis weight 50-90 g/ m² (even up to 240 g/ m²), Bendtsen roughness 250-400 ml/min, brightness 86-92%, and opacity 83-98%.

Coated printing papers based on chemical pulp (WFC) have coatings fluctuate over a wide range according to requirements and application. The following are typical values for once and twice coated printing paper based on chemical pulp: once coated basis weight 90 g/ m², Hunter gloss 65-80%, PPS s10 roughness 0.75-2.2 µm, brightness 80-88%, and opacity 91-94%, and twice coated basis weight 130 g/ m², Hunter gloss 70-80%, PPS s10 roughness 0.65-0.95 µm, brightness 83-90%, and opacity 95-97%.

Other papers include, among others, sackkraft, tissue, and wallpaper.

Board making is performed by using chemical pulp, mechanical pulp and/or recycled pulp. Board grades can be divided e.g. in the following main groups according to applications intended therefor.

Corrugated board including a liner and a fluting.

Boxboards used for making boxes, containers. Boxboards include, among others, liquid packaging boards (FBB = folding boxboard, LPB = liquid packaging board, WLC = white-lined chipboard, SBS = solid bleached sulfite, SUS = solid unbleached sulfite).

Graphic boards used for making e.g. cards, folders, files, cases, covers, etc.

As indicated by the foregoing, there is a huge variety of paper and board grades and machines of several different types are used for making the same.

It is an objective of the present invention to provide a method and apparatus for treating coated and uncoated papers and boards in an optimal manner in a process following the actual manufacturing line downstream of slitting, the webs to be treated being narrow, e.g. 0,15-4,5 m, the size of finishing machines being thus designed respectively to be substantially smaller than the processing equipment normally present in the manufacturing line.

In order to accomplish the objectives of the invention, a method of the invention is characterized by what is set forth in claim 1.

A metal belt calender, which allows for the use of a very extensive pressure range and application time (heat transfer time and/or treating time) in a treatment zone, one and the same apparatus being applicable for the treatment of numerous different coated and uncoated printing papers and boards, has been described in more detail e.g. in earlier applications PCT/Fl03/00066, PCT/Fl03/00067 and PCT/Fl03/00068 of the applicant for present application, and thus it is not described further at this time. I n a metal belt calender, the length of a treatment zone is determined by means of the disposition of belt guiding elements and/or the design and/or disposition of counter-elements, and the contact pressure applied to a web within the treatment zone can be made adjustable for example within the range of about 0.01 MPa to about 200 MPa.

The size of a metal belt calender can be made smaller when using it the treatment of rolled-up narrow fibrous webs adapted to the width of a printing press or some other further processing machine. The use of a metal belt calender enables a rapid change of treatment conditions, allowing e.g. for the manufacture of paper and board grades for different applications on the basis of one and the same stock, said stock possibly consisting of a coated or uncoated web of paper or board. Hence, a switch between grades can be implemented readily and quickly, enabling the manufacture of even small batches in a cost effective fashion. I n addition, the stock purchase costs of a printing house will be reduced.

Furthermore, metal belt calendering stabilizes the structure of a fibrous web, enabling the minimization of bubbling in a printing press resulting from the use of a water-soluble printing ink.

A method of the invention can also be accompanied by a relatively light treatment of the printed fibrous web with a metal belt calender downstream of the printing press, if such treatment is beneficial for polishing the print.

In association with a metal belt calender can also be provided elements for coating a fibrous web, such as for example a dry coating apparatus or a separate coater, upstream or downstream of the metal belt calender. In association with a printing press can be provided not only metal belt calenders but also other types of calenders for enabling a versatile treatment of the fibrous web prior to passing it to the printing press.

A metal belt calender can also be used for drying a fibrous web, thus enabling the use of a higher rolling-up moisture on the papermaking line.

## Claims

1. A method for treating a fibrous web downstream of slitting, wherein the fibrous web is subjected to a finishing treatment for providing the web with desiread properties, wherein the finishing treatment is performed by using one or more finishing units, at least one of which comprises a web processing apparatus provided with a metal belt, said metal-belt equipped web processing apparatus comprising a metal belt calender and/or a metal belt coater and/or a metal belt dryer and/or a dry coater, wherein the finishing treatment is performed at a printing site for providing the fibrous web with a desired finish prior to passing it to a printing press, and wherein said one or more finishing units are disposed on-line with respect to the printing press.

2. A method as set forth in claim 1,
**characterized in that**
the method comprises using a common stock to produce various grades for various applications by varying the running conditions of a metal belt calender.

3. A method as set forth in claim 1,
**characterized in that**
the method also comprises treating the fibrous web with a metal belt calender downstream of the printing press for polishing the print.

## Patentansprüche

1. Verfahren zum Behandeln einer Faserstoffbahn nach einem Längsschneiden, wobei die Faserstoffbahn einer Endbearbeitungsbehandlung zum Versehen der Bahn mit gewünschten Eigenschaften unterzogen wird, wobei die Endbearbeitungsbehandlung durch Verwenden von einer oder mehreren Endbearbeitungseinheiten ausgeführt wird, wobei wenigstens eine von diesen Einheiten ein Bahnbearbeitungsgerät aufweist, das mit einem Metallband versehen ist, wobei das mit dem Metallband ausgestattete Bahnbearbeitungsgerät einen Metallbandkalander und/oder eine Metallbandstreichmaschine und/oder einen Metallbandtrockner und/oder eine Trockenstreichmaschine aufweist, wobei die Endbearbeitungsbehandlung zum Versehen der Faserstoffbahn mit einer gewünschten Appretur auf einer Druckseite vor einem Weiterleiten zu einer Druckmaschine ausgeführt wird, und wobei die eine oder mehreren Endbearbeitungseinheiten bezüglich der Druckmaschine on-line angeordnet sind.

2. Verfahren nach Anspruch 1,
**dadurch gekennzeichnet, dass**
das Verfahren ein Verwenden eines gewöhnlichen Ganzstoffs aufweist, um verschiedene Güteklassen für verschiedene Anwendungen durch Variieren der Arbeitszustände eines Metallbandkalanders herzustellen.

3. Verfahren nach Anspruch 1,
**dadurch gekennzeichnet, dass**
das Verfahren auch ein Behandeln der Faserstoffbahn mit einem Metallbandkalander nach der Druckmaschine zum Polieren des Drucks aufweist.

## Revendications

1. Procédé destiné à traiter une bande fibreuse en aval d'une opération de refente, dans lequel la bande fibreuse est soumise à un traitement de finition pour pourvoir la bande de propriétés désirées, dans lequel le traitement de finition est réalisé en utilisant une ou plusieurs unités de finition, au moins l'une d'entre elles comprenant un appareil de traitement en continu pourvu d'une courroie métallique, ledit appareil de traitement en continu pourvu d'une courroie métallique comprenant une calandre à courroie métallique et/ou une coucheuse à courroie métallique et/ou un sécheur à courroie métallique et/ou une coucheuse à sec, et dans lequel le traitement de finition est réalisé au niveau d'un site d'impression pour pourvoir la bande fibreuse d'une finition désirée avant de la faire passer à la machine d'impression, et dans lequel lesdites une ou plusieurs unités de finition sont disposées en ligne par rapport à la machine d'impression.

2. Procédé selon la revendication 1,
**caractérisé en ce que**
le procédé comprend d'utiliser un stock courant pour produire diverses qualités destinées à diverses applications en faisant varier les conditions de fonctionnement d'une calandre à courroie métallique.

3. Procédé selon la revendication 1,
**caractérisé en ce que**
le procédé comprend aussi de traiter la bande fibreuse avec une calandre à courroie métallique en aval de la machine d'impression pour polir l'impression.
